

## UNITED STATES PATENT OFFICE

2,321,307

## LUBRICATING OIL, INSULATING AND SIMILAR OIL

Louis A. Mikeska, Westfield, and Eugene Lieber, Linden, N. J., assignors to Standard Oil Development Company, a corporation of Delaware

No Drawing. Application August 17, 1937,  
Serial No. 159,504

18 Claims. (Cl. 252—37)

This invention relates to an improvement in lubricating, insulating and similar oils. It particularly relates to the improvement of the stability of oils and prevents their decomposition, especially at elevated temperatures under the extreme oxidizing conditions existing in internal combustion engines, by the addition of oxidation inhibitors and sludge dispersers of the class of alkyl phosphites and aryl phosphites having the formula  $P(TR)_3$  in which T represents sulphur, selenium or tellurium and R represents an alkyl or an aryl radical.

Motor oils and other lubricants which are subjected to use at elevated temperatures show deterioration by oxidation, sludge formation and the like. Such deterioration may be checked and the lubricating oil considerably improved by the addition of certain oxidation inhibiting agents and the addition of agents for inhibiting sludge formation and the like. Thus it is already known that lubricating oils can be improved in respect to any particular property by the addition of small amounts of a particular substance. However, most of these agents which are useful for one particular purpose as, for instance, to inhibit oxidation, are undesirable in that such agents tend to increase undesirable characteristics of the oil in other respects as, for example, sludge formation.

In the present case an entirely new group of substances have been discovered which impart desirable oxidation inhibiting properties to a lubricating oil, thereby rendering it stable under all temperature conditions at which the lubricant is employed. This class of oxidation inhibitors not only does not increase the sludge formation but it actually also acts as a sludge disperser.

These compounds are of the class of alkyl and aryl phosphites containing a member of the sulphur family as, for example, trihexyl thiophosphite, triamyl thiophosphite, tributyl thiophosphite, triamyl selenothiophosphite, trialkyl tellurophosphite, triphenyl thiophosphite, tritolyl thiophosphite, trinaphthyl thiophosphite, or a mixture thereof. The alkyl radical may contain substituted groups as, for instance, chlorine, or the aryl radical may be alkylated with an alkyl group, containing preferably 3 to 12 carbon atoms in the alkyl group, as for example triamyl phenyl thiophosphite and tributyl phenyl thiophosphite, or the aryl radical may contain other substituted groups.

Compounds such as monoalkyl thiophosphites and dialkyl thiophosphites, as for example monoamyl thiophosphite, and dibutyl thiophosphite, are also satisfactory but it is preferred to use the trithio alkyl compounds. The preferred thiophosphite compounds are alkyl thiophosphites having from 3 to 20 carbon atoms in the alkyl group, especially those having from 4 to 6 carbon

atoms in the alkyl group and those alkyl thiophosphites which have boiling points above 125° C. These thiophosphites may also contain mixed alkyl groups such as monoamyl di-butyl thiophosphites and di-amyl monohexyl thiophosphites. A mixed alkyl aryl compound may be used as, for example, monoamyl diphenyl thiophosphite.

These compounds may be prepared by any of 10 well known methods. For example, an alkyl mercaptan such as amyl mercaptan may be reacted with phosphorous acid in the presence of hydrocarbon solvents at a temperature of about 150° C. and a pressure of one atmosphere. The 15 thiophosphites may be separated from the reaction mixture by simply distilling off the solvents under reduced pressure, if necessary. One suitable method of preparing the thiophosphites is given by the following example:

20 A two-way flask was fitted with a dropping funnel and a return condenser. The flask was charged with 104 grams of amyl mercaptan and 230 cc. of ethylene di-chloride, 40 grams of phosphorus trichloride was then slowly added through 25 a dropping funnel, while refluxing the solution. The heating was continued for four hours at the end of which time the evolution of hydrochloric acid ceased. The solvent was removed by heating the reaction product at 100° C. under reduced pressure. Approximately 80 to 85 grams of the colorless amyl thiophosphite was recovered from the flask. This product was tested and gave a negative reaction to doctor solution, thus indicating that no free mercaptans were present.

30 35 The thiophosphites may also be prepared without the use of a solvent and compounds such as pyridine may be added to the mixture to increase the speed of the action. The crude thiophosphites may be further purified in any desired manner as, for example, by solvent extraction or distillation.

40 45 These thiophosphites, free from impurities, may be added to any type of mineral oil. The oil may be synthetic or a natural oil refined by any of the known methods as, for example, by acid, alkali or clay treating by solvent extraction, hydrogenation or destructive hydrogenation, or by a combination of any of the foregoing. The alkyl thiophosphites give particularly desirable results 50 when added to a lubricating oil of predominantly paraffinic nature.

55 The amount of the thiophosphite added may vary considerably with the character of the particular oil and may also vary depending upon the conditions under which the particular oil is to be subjected in operation. As little as 0.01% may be effective but it is preferred to use from 0.2% to 0.5% and as high as 5% may be used. As a general rule, it is found that 1% more or less gives 60 satisfactory results. Other compounds may also

be included in the blend as, for instance, dyes, pour point depressors, oiliness agents, sludge dispersers and other ingredients.

An example of the present invention is shown by the following example:

Triamyl thiophosphite was blended with a well refined mineral oil S. A. E. 20 in the proportion of 0.2% and the following tests were run on the blend and on the blank oil not containing the triamyl thiophosphite:

#### Cone test

A method for determining the tendency of an oil to deposit sludge matter upon a heated metallic surface. It consists in slowly dropping the oil to be tested over a heated metal cone which is generally steel. The cone is a circumferential groove milled out in a screw fashion on the periphery thereby allowing a time of contact of about one minute between the heated steel surface and the oil. A total volume of 60 cc. of oil is released from a dropping funnel over a period of two hours. The temperature of the cone may be any desired value but for lubricating oils it is preferred to use about 250° C. since it represents approximately the extreme temperature to which oils are ordinarily exposed in the internal combustion engine. After the entire volume of oil is run over the metallic surface the cone is washed with naphtha to completely remove the adhering oil without disturbing the deposit left on the cone. The cone is then weighed and the increase in weight of the cone due to the deposit left thereon by the oil is expressed in milligrams.

#### Sligh test

This determines the tendency of an oil to sludge under oxidizing conditions as described in the A. S. T. M. report committee D2, page 22, 1927, except that the time of run was increased from 2½ hours to 24 hours in order to secure a more accurate test and comparison.

#### Lead tolerance

This test is a measurement of the amount of lead oleate which may be added to a lubricant without causing it to assume definite corrosive properties when run on the Underwood corrosion testing apparatus. The Underwood test is conducted as follows:

1500 cc. of the oil being treated is maintained at 325° F. and sprayed for 5 hours against 2 each of copper-lead and cadmium-silver alloy bearings such as are used on automobile engines. The oil is circulated from a sump through a heating tube to a gear pump and thus by means of jets, maintained at a constant temperature on the 4 half bearings of cadmium-silver and copper-lead. The oil drippings from the bearings are recirculated. The bearings are weighed before and after the test to determine any loss in weight. The tests are then repeated with the addition of lead oleate in increments of 0.005% by weight (calculated as lead oxide). When the test results in the loss of weight equivalent to 1% of the weight of the bearing, the oil is said to be corrosive and it indicates that the lead tolerance of the oil has been exceeded and the amount of lead oxide added in the last previous test is regarded as the lead tolerance. By correlation of this test with the use of highly refined lubricating oil in actual operation of automobile engines under service conditions, it has been determined that a lead tolerance below 0.020 is unsatisfactory.

#### Oxidation rate

A test to determine the tendency of the oil to oxidize. Oxygen is bubbled in a close circulatory system through 10 cc. of the respective oils which are held at a temperature of 200° C. At 15 minute intervals the amount of oxygen remaining unconsumed is measured and the volume of oxygen absorbed by the oil calculated by differences.

10 The data on the blend of triamyl thiophosphite with the mineral oil S. A. E. 20 as compared with the blank oil secured by running the above described tests is as follows:

|                                                      | Cone deposit, gr.                 |
|------------------------------------------------------|-----------------------------------|
| 15 S. A. E. 20 mineral oil                           | 0.40                              |
| S. A. E. 20 mineral oil + 0.2% triamyl thiophosphite | 0.22                              |
|                                                      | Slight No.                        |
| 20 S. A. E. 20 mineral oil                           | 39                                |
| S. A. E. 20 mineral oil + 0.2% triamyl thiophosphite | 37.7                              |
|                                                      | Lead tolerance                    |
| 25 S. A. E. 20 mineral oil                           | 0.005                             |
| S. A. E. 20 mineral oil + 0.1% triamyl thiophosphite | 0.030                             |
|                                                      | Volume of oxygen absorbed, 10 cc. |
| 30 Sample, 15 minute interval at 200° C.             |                                   |
| S. A. E. 20 mineral oil                              | 155 70 — —                        |
| S. A. E. 20 mineral oil + 0.2% triamyl thiophosphite | 88 56 40 —                        |

35 The invention is not to be limited by any theory or method of operation but only by the following claims in which it is desired to claim all novelty in so far as the prior art permits.

We claim:

1. An improved lubricant for use in internal combustion engines comprising a refined hydrocarbon oil containing an effective concentration below about 1% of an oxidation inhibitor effective in preventing decomposition of said oil at the elevated temperatures encountered in lubricating internal combustion engines, said oxidation inhibitor being a compound of the class of organic phosphites containing an element selected from the class consisting of sulfur, selenium and tellurium, said element being attached directly to the phosphorus and the organic group, the organic radicals of the said organic phosphites having 3 to 20 carbon atoms in each radical and being selected from the group consisting of alkyl radicals and halogen substituted alkyl radicals.
2. A lubricant according to claim 1 in which the oxidation inhibitor has the formula



in which T represents an element selected from the group consisting of sulfur, selenium and tellurium, and R<sub>1</sub>, R<sub>2</sub>, and R<sub>3</sub> represent organic radicals selected from the group consisting of alkyl radicals and halogenated substituted alkyl radicals.

3. A lubricant according to claim 1 in which the oxidation inhibitor has the formula P(T alkyl group)<sub>3</sub>, in which T represents an element selected from the group consisting of sulfur, selenium and tellurium.
4. An improved lubricant for use in internal

combustion engines comprising a refined hydro-carbon oil containing 0.1 to 1% of an oxidation inhibitor effective in preventing decomposition of such oils at the elevated temperatures encountered in lubricating internal combustion engines, said oxidation inhibitor having the formula  $P(T\text{ alkyl group})_3$ , in which T represents an element selected from the group consisting of sulfur, selenium and tellurium, and in which the alkyl group contains from 4 to 6 carbon atoms.

5. An improved lubricant for use in internal combustion engines comprising a refined hydro-carbon oil containing an effective concentration below about 1% of an oxidation inhibitor effective in preventing decomposition of said oil at the elevated temperatures encountered in lubricating internal combustion engines, said oxidation inhibitor having the formula  $P(S\text{ alkyl group})_3$ , in which the alkyl group contains from 4 to 6 carbon atoms.

6. A lubricant according to claim 5 in which the concentration of the oxidation inhibitor is from 0.2 to 0.5%.

7. An improved lubricant for use in internal combustion engines comprising a refined hydro-carbon oil containing an effective concentration below about 1% of an oxidation inhibitor effective in preventing decomposition of said oil at the elevated temperatures encountered in lubricating internal combustion engines, said oxidation inhibitor having the formula  $P(S\text{ alkyl group})_3$ , and having a boiling point above 125° C.

8. A method of lubricating an internal combustion engine which comprises introducing into the crank case of said engine a refined hydro-carbon oil containing from 0.01 to 1% of an oxidation inhibitor of the formula



in which T represents an element selected from the group consisting of sulfur, selenium and tellurium, and  $R_1$ ,  $R_2$ , and  $R_3$  represent organic radicals having 3 to 20 carbon atoms in each radical and selected from the group consisting of alkyl radicals and halogen substituted alkyl radicals.

9. A method of lubricating an internal combustion engine which comprises introducing into the crank case of said engine a refined hydro-carbon oil containing from 0.2 to 0.5% of an oxidation inhibitor of the formula  $P(S\text{ alkyl group})_3$ , in which the alkyl group contains from 4 to 6 carbon atoms.

10. A lubricating oil containing lead oleate in an amount sufficient to corrode alloy bearings in the absence of an oxidation inhibitor, and an oxidation inhibitor in an amount sufficient to prevent such corrosion, said oxidation inhibitor having the formula



in which T represents an element selected from the group consisting of sulphur, selenium and tellurium, and  $R_1$ ,  $R_2$ , and  $R_3$  represent organic radicals each having 3 to 20 carbon atoms and

selected from the group consisting of alkyl radicals and halogen substituted alkyl radicals.

11. A lubricating oil containing lead oleate in an amount sufficient to corrode alloy bearings in the absence of an oxidation inhibitor, and tri-  
amyl thiophosphite in an amount sufficient to prevent such corrosion.

12. A lubricating oil containing a soap of an acid which tends to cause corrosion of alloy bearings in the absence of an oxidation inhibitor, and an oxidation inhibitor in an amount sufficient to prevent such corrosion, said oxidation inhibitor having the formula



in which T represents an element selected from the group consisting of sulfur, selenium and tellurium, and  $R_1$ ,  $R_2$  and  $R_3$  represent organic radicals each having 3 to 20 carbon atoms and selected from the group consisting of alkyl radicals and halogen substituted alkyl radicals.

13. A lubricating oil containing a lead soap in an amount sufficient to corrode alloy bearings in the absence of an oxidation inhibitor, and an oxidation inhibitor in an amount sufficient to prevent such corrosion, said oxidation inhibitor having the formula



in which T represents an element selected from the group consisting of sulfur, selenium and tellurium, and  $R_1$ ,  $R_2$  and  $R_3$  represent organic radicals each having 3 to 20 carbon atoms and selected from the group consisting of alkyl radicals and halogen substituted alkyl radicals.

14. A lubricating oil containing a lead soap in an amount sufficient to corrode alloy bearings in the absence of an oxidation inhibitor, and triamyl thiophosphite in an amount sufficient to prevent such corrosion.

15. An improved lubricant according to claim 7 in which each of the said alkyl groups of the oxidation inhibitor contains not more than 6 carbon atoms.

16. A lubricating oil non-corrosive to hard metal alloy bearings comprising a mineral lubricating oil normally corrosive to said bearings and an alkyl thiophosphite having 3 to 6 carbon atoms in each alkyl radical, said alkyl thiophosphite being added in a small but sufficient quantity to inhibit the corrosion to said hard metal alloy bearing.

17. A lubricating oil as described in claim 16 in which the alkyl thiophosphite is tri-amyl tri-thiophosphite.

18. The method of preventing corrosion of bearing metal alloys selected from the group consisting of cadmium-silver alloys and copper-lead alloys in the presence of highly refined lubricating oils in internal combustion engines which comprises adding to said lubricating oils an alkyl thiophosphite having 3 to 6 carbon atoms in each alkyl radical in a small but sufficient amount to inhibit said corrosion.

LOUIS A. MIKESKA.  
EUGENE LIEBER.